

## UNITED STATES PATENT OFFICE

WILHELM PFAFFENDORF, OF HOCHST-ON-THE-MAIN, GERMANY, ASSIGNOR, BY MESNE ASSIGNMENTS, TO GENERAL ANILINE WORKS, INC., OF NEW YORK, N. Y., A CORPORATION OF DELAWARE

## PROCESS OF DEGREASING TEXTILE MATERIALS

No Drawing. Application filed May 23, 1927, Serial No. 194,533, and in Germany June 14, 1926.

My present invention relates to a process of degreasing textile materials.

There has been disclosed in numerous patents processes of degreasing textile material in which organic solvents are used for this purpose. None of the proposed solvents perfectly meets the indispensable requirements, namely: the protection of the fibers against deterioration; economy; avoidance of damage to the apparatus, and property of being fireproof. The chlorinated hydrocarbons hitherto used for this purpose offer the advantage of being incombustible, and with almost all of them the extraction of fat can be effected under suitable conditions, while the fibers are largely protected against deterioration by the degreasing process. Nevertheless, the use of the said hydrocarbons has not been generally adopted for the purpose in question, as the members of this class of bodies boiling at a temperature below 50° C. are causing great losses of the solvents owing to their volatility, and because the higher-boiling members, under the conditions used in practice, strongly attack the apparatus, especially those made of iron.

Now I have found that the ethylene chloride  $\text{CH}_2\text{Cl}=\text{CH}_2\text{Cl}$ , in spite of its boiling point of above 80° C., is extremely stable towards the action of water vapor and oxygen, even in the presence of metals, metal oxides, of bodies having a large surface and other bodies of a catalytic action. It is a perfect degreasing agent, which protects the material to be scoured against deterioration, does not attack the apparatus, is not liable to take fire and allows an extensive recovery of the solvent used.

The following example serves to illustrate my invention, but it is not intended to limit it thereto:

In an extractor of 8 ccm. capacity 800 kg. of raw wool are washed at a temperature of 60° C. with ethylene chloride until the liquid flowing off is free from grease, which occurs in a very short time. The solvent is then run off at the bottom, and the portions left in the wool are eliminated therefrom by flooding the material with hot water.

The temperature depends on the materials and may vary between 0° C. and 80° C.

## I claim:

The process which comprises washing textile materials with ethylene chloride 55  $\text{CH}_2\text{Cl}=\text{CH}_2\text{Cl}$  at a temperature between about 0° C. to about 80° C.

In testimony whereof I have hereunto set my hand.

WILHELM PFAFFENDORF. 60

65

70

75

80

85

90

95

100